

## 1

3,598,514

## METHODS OF APPLYING SOIL-RELEASE COMPOSITIONS TO TEXTILE MATERIALS

Stephen B. Sello, Cedar Grove, Illo Emil Pensa, Palisades Park, and Bipinchandra R. Shukla, East Paterson, N.J., assignors to J. P. Stevens and Co., Inc., New York, N.Y.

No Drawing. Filed Feb. 27, 1969, Ser. No. 803,045  
Int. Cl. D06m 13/12

U.S. CI. 8—115.6

5 Claims

## ABSTRACT OF THE DISCLOSURE

Textile materials containing substantial proportions of cellulosic and/or hydrophobic constituents are provided with both durable-press and soil-release properties by depositing on said textile materials acid catalyzed durable-press resin precursor; polyether derivative selected from the group consisting of polyalkylene glycols, the mono- and di-fatty acid esters of polyalkylene glycols, and the mono- and di-alkyl ethers of polyalkylene glycols, and their mixtures; fluorocarbon polymer, and a catalytic quantity of acidic catalyst. The fluorocarbon polymer contains highly fluorinated oleophobic and hydrophobic portions and nonfluorinated hydrophilic portions.

This invention concerns improved methods and compositions for imparting soil-release characteristics to textile substrates which are to have a "durable-press" or "permanent-press" finish.

More particularly, this invention relates to compositions comprising fluorocarbon polymers and polyether derivatives, which when used in conjunction with durable-press resin precursors, catalysts and optional textile adjuvants, produce a finish having good soil-release upon one laundering, without compromising the durable-press finish.

With the advent of "wash-and-wear," "durable-press" or "permanent-press" garments, the utilization of synthetic fibers and their blends with cellulosics and/or other natural fibers has become widespread. Garments containing substantial quantities of polyesters and other hydrophobic fibers have been particularly favored because they strengthen the abrasion resistance of cellulosic based garments and increase the crease resistance of the garments without the need of an increased amount of cross-linking resins. Unfortunately, garments containing a substantial quantity of these synthetic fibers (as illustrated by polyester) have exhibited a pronounced tendency to retain soil and stains, particularly oily stains. Furthermore, these fabrics or garments have been found to resist release of the soil or stains even upon exposure to repeated laundering. In all likelihood the propensity of these blends of synthetic and natural fiber to accumulate stains is due to the inherently oleophilic structure of synthetics such as polyester.

Increased resistance to the release of soil and stains also results from the crosslinking resins employed to impart durable-press properties to fabrics. These resins are probably converted during their insolubilization to oleophilic structures. Whatever the factors that are involved, soil and stain retention in fabrics treated with thermoset crosslinking resins has been a serious and costly problem.

U.S. Pat. No. 3,377,249, discloses a process for im-

## 2

parting soil release finishes to textile materials containing polyester fibers. The claimed process comprises applying an aminoplast textile resin and a synthetic acid emulsion polymer and curing the textile resin to impart the desired finish.

The finishing system of the above patentee is deficient in an important aspect, namely, that at least two launderings are required to remove oily soil or stains.

In order to overcome this problem, applicants have developed a finishing system for textiles which contains relatively small quantities of fluorocarbon polymers and certain polyether derivatives. The finishing system also includes durable-press resin precursors such as are disclosed in the U.S. Pat. No. 3,377,249. Not only are initial soil-release properties excellent, but the finish is durable, crease retention is excellent and the hand of the finished product is satisfactory. Inasmuch as the improvement in soil release upon one laundering is obtained at application levels where the individual components of the finish (fluorocarbon polymer and polyether derivative) are ineffective in removing lubricating oil type of stains, the results are most unexpected. Even more startling, good initial and long-term soil release have been obtained in the complete absence of the acrylic acid type polymer component of the soil-release finish said by U.S. Pat. No. 3,377,249 to be critical to acceptable soil release. In view of this, applicants' invention is contrary to the teaching of the prior art.

In practicing the present invention, samples of the textile substrate are treated with a composition comprising durable-press resin precursor, fluorocarbon polymer, polyether derivative, textile adjuvants and necessary catalysts to obtain the desired pickup level. The treated samples are dried between about 60° C. to 130° C., desired configurations imparted therein and the configured samples set by exposure to heat and pressure. The setting step is followed by curing at a sufficiently elevated temperature and for a sufficiently long time to cure the durable-press resin precursor. The cured substrate has long-lasting durable-press and soil-release properties.

In preferred practice, the textile substrate is padded in an aqueous bath comprising 0.1 to 2% by weight of fluorocarbon polymer, 3 to 15% by weight of polyether derivative, 4-20% by weight of durable-press resin precursor and 0.1 to 5% by weight of acid catalyst. After padding, the treated substrate is passed through squeeze rollers set at about 30-50 lbs./sq. inch so that the desired "add-on" of each component (based upon the weight of the substrate) is present upon drying. The substrate is then dried at about 90° C. to 120° C. until a moisture content of from about 2 to 11% by weight moisture is obtained. The substrate is placed in the desired configuration and then pressed and cured using the conditions commonly employed in producing creased durable-press garments.

While it is convenient to apply all the components of the padding bath simultaneously, the components can be applied separately or in more than one bath.

The fluorocarbon polymers which are an essential component of the soil-release compositions of this invention contain highly fluorinated oleophobic and hydrophobic portions and nonfluorinated hydrophilic portions. Preferably, the highly fluorinated portions contain perfluoroalkyl groups of at least 4 carbon atoms and the non-fluorinated portions contain groups of the formula  $(C_xH_{2x}O)_e$  where  $x$  is an integer of 1 to 4 and  $e$  is an

integer of 4 to 20. Illustrative of suitable fluorocarbon polymers are:

(a) A homopolymer of a monomer of the formula



wherein

$R_f$  is a fluoroalkyl radical containing 4 to 25 carbon atoms such as



wherein

$Z$  is H or F, and

$m$  is an integer ranging from 3 to 24,

$X$  is a difunctional radical selected from the group consisting of



wherein

$R$  is lower alkyl (from 1 to 4 carbon atoms),

$b$  is an integer ranging from 0 to 15,

$g$  ranges from about 1 to 4,

$e$  is an integer ranging from 4 to 20,

$G$  is an unsaturated acyl radical



wherein

$R'$  is an unsaturated aliphatic radical containing from 2 to 8 carbon atoms, and

$Y$  is  $[-C_xH_{2x}O-]$ , wherein  $x$  is an integer ranging from 1 to 4, and

(b) Copolymers of:



wherein

$R_f$ ,  $X$ ,  $G$ ,  $e$  and  $Y$  are as defined above, with at least one of vinylic monomers such as vinyl chloride, vinyl acetate, ethylene, propylene, acrylic acid, methacrylic acid, acrylate or methacrylate esters, fluorinated acrylic esters, or acrylates or methacrylates of polyethylene oxide ( $CH_2CH_2O$ ) groups and

(c) Commercially available fluorinated polymer having an average composition represented by the formula



Outstanding results are obtained with fluorocarbon polymers prepared from monomers of the formula:



wherein

$R^4$  is a perfluoroalkyl radical having 6 to 10 carbon atoms,

$R^2$  is hydrogen or lower alkyl having from 1 to 6 carbon atoms,

$d$  ranges from about 12 to 20, and

$R^3$  and  $R^4$  are selected from the group consisted of hydrogen and lower alkyl having from 1 to 4 carbon atoms.

The fluorocarbon polymers can be prepared following known procedures such as disclosed in the following patents.—U.S.: 2,732,398; 2,803,615; 2,915,554; British: 857,689.

The following are specific illustrations of the preferred fluorocarbon monomers:



The polyether derivatives suitable for the soil-release compositions include polyalkylene glycols (such as polyethylene and polypropylene glycols), the mono- and di-fatty acid esters of polyalkylene glycols (such as the mono- and di-oleates and stearates of polyethylene glycol) and the mono- and di-alkyl ethers of polyalkylene glycols (such as the mono- and dimethyl and ethyl ethers of polyethylene glycol).

The textile substrates used in the present invention are textile materials containing substantial quantities of natural and/or synthetic hydrophobic thermoplastic materials in the form of yarns, slivers, filaments, tows, fibers, articles, garments and the like produced by processes such as drawing, spinning, combing, weaving, knitting, needle-punching or other non-weaving procedures. Illustrative of these substrates are cellulosics such as cotton; and synthetic polymers such as polyesters, polyamides, polyethylene, polypropylene, polyacrylonitrile or blends of these cellulosics and synthetics. The process has considerable utility in imparting a soil-release finish to textile materials containing at least 25% by weight of these synthetics, usually from 50% by weight and upwards. The favored synthetic

substrate is polyester such as poly(ethylene terephthalate) and poly(1,4-cyclohexylene - dimethylene terephthalate). When the substrate comprises 100% by weight of synthetic fibers the durable-press resin precursor can be omitted.

Durable-press characteristics are obtained by the use of acid catalyzed durable-press resin precursors which can be generically grouped as adducts of formaldehyde with amides. The products can be linear or cyclic in structure or they can comprise mixtures of one or more of these structural types. These precursors can be aliphatic, aromatic

or heterocyclic. A listing of preferred resin precursors includes:

$N^2,N^4,N^6$ -tris(hydroxymethyl) melamine, hexakis(methoxymethyl) melamine, the bis(hydroxymethyl) triazolidinones,

1,3-bis(hydroxymethyl)urea, 1,3-bis(hydroxymethyl)-2-imidazolidinone,

4,5-dihydroxy-1,3-bis(hydroxymethyl)-2-imidazolidinone,

$N,N^1$ -bis(methoxymethyl)uron,

2-methoxyethyl  $N,N$ -bis(hydroxymethyl) carbamate and dimethyloldihydroxy ethylene urea, among others.

Preferred acidic catalysts for said resin precursors include metal salts such as magnesium chloride, zinc nitrate and zinc fluoroborate; and amino salts such as monoethanolamine hydrochloride and 2-amino-2-methylpropanol nitrate.

The various modifiers, agents, conditioners and acids which alter characteristics other than durable press and stain release of the finished textile products are generally categorized as textile adjuvants. These adjuvants include softeners, surfactants, hand modifiers, antistatics, thickeners and the like. Illustrative of these are polyvinyl acetates of various average molecular weight ranges, thickeners such as the natural gums, ethylated starches, hydroxyethylcellulose and sodium carboxymethylcellulose, among others. Also intended to be included as adjuvants are the various wetting agents and other surfactants such as p-(1,1,3,3-tetramethylbutyl)phenoxyethoxyethanol, the sodium salt of N-methyl-N-oleyltaurine, and the sodium salts of sulfonated hydrocarbons, among others. Since the role of the textile adjuvants is not critical to the inventive process, no attempt has been made to present an exhaustive or even lengthy list. Voluminous listings of the many textile adjuvants can be found in commercial brochures, chemical literature and in the soap and chemical specialties listings of the Department of Agriculture.

All of the constituents of the process of this invention can be applied to the textile substrates by any of the conventional impregnation methods known in the textile art. These include the preferred padding or dipping method, as well as spraying, coating, or the like. The polymeric treating compositions can be in the form of a solution where the solubility characteristics allow it, or in the form of an emulsion or dispersion. Preferably, the textile substrate is dipped into a bath which is an aqueous dispersion of the components to be applied.

The concentrations of the treating agents employed are varied to some extent according to the effect sought, the type of substrate, and the weight of the substrate. The following data show the ranges of components to be added in terms of parts by weight per 100 parts by weight of original fabric (this basis for indicating the weight of finish component added being hereinafter referred to as "Percent Solids OWF").

| Component                          | Percent solids OWF |                 |
|------------------------------------|--------------------|-----------------|
|                                    | Suitable range     | Preferred range |
| Fluorocarbon polymer.....          | 0.1-3.0            | 0.15-0.5        |
| Durable-press resin precursor..... | 3.0-20.0           | 5.0-10.0        |
| Polyether derivative.....          | 2.0-15.0           | 3.0-8.0         |
| Acid catalyst.....                 | 0.1-20.0           | 0.2-6.0         |

The particular heating temperatures and the length of the heating cycle are not critical as long as the combination of heating temperature and time is sufficient to accomplish the drying, setting of configuration or curing of the durable-press resin precursor, etc. For example, after application of the soil-release composition the treated textile article can be dried up to the curing temperature of the resin precursor.

Similarly, the setting of the crease or pleat can be accomplished using different combinations of temperature, time and pressure. For instance, the treated fabric after being made into a garment can be pressed on an electrically heated hot-head garment press as follows: Steam is used for the first 5 seconds (at 150 to 160° C.), then the temperature is raised between about 160° C. to 250° C., keeping the head pressure at about 85-100 pounds/sq. inch. After the final heating, vacuum is applied for from about 3 to 15 seconds or higher to complete the pressing operation. Curing is accomplished by heating between about 130° C. to about 200° C.

If desired, the setting operation can be accomplished in a garment-setting oven using comparable temperatures and times. Again as the mode of pressing and setting the creases or pleats is not novel nor critical to the invention, no attempt will be made to describe them in detail.

In order to illustrate the invention as completely as possible, the accompanying examples are submitted. Unless otherwise specified, all percentages are expressed on

a weight basis. A description of the test methods and the terms used in the examples precedes the examples.

#### EVALUATION OF SOIL RELEASE

5 The following soiling agents were used, denoted respectively as vegetable oil (V), mineral oil (M), and lubricating oil (L):

10 Corn oil.—(Not hydrogenated); e.g., "Mazola," Best Foods Division, Corn Products Co., New York, N.Y.

15 Extra heavy mineral oil.—Saybolt viscosity between 360 and 390 at 100° F., specific gravity between 0.880 and 0.900 at 60° F.; e.g., "Nujol," Plough, Inc., New York, N.Y.

15 Used, dirty lubricating oil.—Drained from the crank-case of an automobile.

20 The fabric specimen, no smaller than 18 by 15 inches, was laid on a glass plate covered by polyethylene film 3 inches square. The soiling agent was applied to the face side, using 4 drops (0.25 ml.) when in liquid form.

25 A 1.2 ml. (0.25 teaspoon) portion is spread as a circular spot approximately 2.4 cm. in diameter, but not worked into the fabric. Polyethylene film 3 inches square was placed over the spotted area immediately, and a 2.5-inch diameter, 5-pounds weight was left over each spot for 30 seconds to impart a pressure of approximately 1

30 pound per square inch. Then the original polyethylene films were discarded, and the specimen was sandwiched between two paper towels, the sandwich having been covered top and bottom with polyethylene film to prevent soiling the glass plate and the weight. The 5-pound weight was then placed over the spotted area for 3 seconds to blot out excess soiling agent. (If excess soiling agent remained, it was removed at once by lightly blotting with a facial tissue.) Next, stained specimens were aged in the ordinary room atmosphere for at least 30 minutes by being hung so there was no contact between specimens.

35 Laundering was done in a home-type washer at approximately 50° C. in 5-pound loads using the high water level (16 gallons) with a level cupful of non-ionic detergent, and tumble dried.

40 Rating for residual soil used the Deering Milliken Photographic Standards for Evaluation of Soil-Release Finishes, the scale of which is from 1 to 5. No visible spot remaining was denoted by 5, and a spot barely visible by 4, with 3, 2, and 1 denoting progressively serious strains. The evaluation was made under ordinary overhead fluorescent room lighting of normal intensity with the test specimen flat on a table top  $35 \pm 5$  inches from the floor directly under the light, and viewed from all possible angles. The rating for each stain was the lowest number assigned it from any angle.

45 Evaluation of wash and wear.—AATCC 88A-1964T Test III-C for laundering: Home-type washer, 5-pound load, full cycle, 60° C., synthetic detergent; tumble drying (TD). The number of laundering-drying cycles (as 1, 2 or 5) is indicated in tables by 1L, 2L, or 5L. The 5-point rating scale extend from 1 (extensively wrinkled) to 5 (perfectly smooth).

50 Evaluation of crease retention.—AATCC 88A-1964T Test III-C also. The rating scale is as follows: 1. (no crease remaining), 2. (slight crease), 3. (moderate crease), 4. (sharp crease), and 5. (unchanged, very sharp crease).

55 OWB.—Means on the weight of the bath used for padding in percent.

60 Percent Solids OWF.—Means parts by weight of finishing component added per hundred parts by weight of original fabric.

65 WPU.—Means wet pickup or percent add-on, i.e.,

70 
$$\frac{\text{Weight of wet add-on} \times 100}{\text{Weight of original fabric}}$$

7  
EMBODIMENT A

A monomer having the structure:



is prepared by the methods described in U.S. Pats. 2,803,615 and 2,915,554.

## 8

bake and 5 seconds vacuum. Finally, the durable-press finish was cured by heating at 165° C. for 15 minutes.

The "wash-and-wear," crease-retention and soil-release data obtained through the use of the individual soil-release components appear in Table 1. The term "Stained after 5L" indicates that after the finishing system was applied, the sample was laundered five times before being stained.

TABLE 1

| Percent OWF <sup>1</sup> | MMF<br>of<br>polymer-<br>active | PEG | Wash<br>and<br>wear<br>(5L-TD) | Crease<br>retention<br>(5L-TD) | Soil release    |     |   |     |                  |   |   |   |   |     |
|--------------------------|---------------------------------|-----|--------------------------------|--------------------------------|-----------------|-----|---|-----|------------------|---|---|---|---|-----|
|                          |                                 |     |                                |                                | Original stains |     |   |     | Stained after 5L |   |   |   |   |     |
|                          |                                 |     |                                |                                | V               | L   | V | L   | V                | L | V | L |   |     |
| 0.18                     |                                 |     |                                |                                | 4.3             | 4.3 | 4 | 1/2 | 4/5              | 2 | 3 | 2 | 4 | 3   |
| 0.14                     |                                 |     |                                |                                | 4.3             | 4.3 | 3 | 1   | 4/5              | 1 | 3 | 1 | 4 | 1/2 |
|                          |                                 | 5.4 |                                |                                | 4.0             | 4.3 | 3 | 2   | 3                | 2 | 2 | 1 | 2 | 1   |
|                          |                                 |     | 5.4                            |                                | 3.5             | 4.0 | 3 | 2   | 3                | 2 | 2 | 1 | 2 | 1   |

<sup>1</sup> The fabric also contained dimethylol dihydroxy ethylene urea (5.7% solids OWF) with zinc nitrate (0.6% solids OWF).

NOTE.—Fabric used: 50/50 polyester/cotton blend twist twill dyed (spruce).

In preparing this monomer, the alcohol



is made in accordance with the procedures of U.S. Pat. 2,915,554 and this alcohol is reacted with acrylic acid in accordance with the procedures of U.S. Pat. 2,803,615. The monomer is emulsion polymerized by the method described in Example 1 of U.S. Pat. 2,803,615. The reaction mixture is cooled and worked up by the described techniques to yield a polymer latex having a solids content of about 36% solids.

## EXAMPLE 1

Unsuccessful attempts to impart a durable soil-release finish using the individual components (fluorocarbon polymer and polyether derivative) of the soil-release finish

The substrate used for treatment is a fabric blend of polyester (50% by weight) and cotton (50% by weight) having a thread count (warp x filling) of 134 x 66, dyed spruce green in color.

The following application procedure was used. Aqueous pad baths were made up containing varying amounts of the individual components of the soil-release composition, the fluorocarbon polymer described in Embodiment A and different polyether derivatives,<sup>1</sup> plus dimethylol dihydroxyethylene urea resin (9.5% solids OWB) and 1.0% solids OWB of  $\text{Zn}(\text{NO}_3)_2$  catalyst. The fabric samples were padded through squeeze rolls set to give a wet pickup of about 60%.

After padding, the fabric sample was framed to the original dimensions and dried at approximately 125° C.

As can be seen from the data in Table 1, the individual components of the soil-release composition (fluorocarbon polymer and the polyether additives) are relatively ineffective in providing a durable stain-release finish that releases oil stains upon one laundering but persists upon repeated laundering. The subsequent examples establish the synergistic effect that is obtained when the fluorocarbon polymer and alcohol additive components are combined.

## EXAMPLE 2

35 A soil-release composition comprising mixtures of fluorocarbon polymer and the monomethyl ether of polyethylene glycol

The fabric substrate used for treatment is the same one employed in Example 1. Pad baths are made up containing two different concentrations of the fluorocarbon polymer of Embodiment A and two different concentrations of the methyl ether of polyethylene glycol, molecular weight 860. Each pad formulation also contained 1.0% OWB zinc nitrate catalyst and 9.5% OWB dimethylol dihydroxyethylene urea resin precursor.

The samples were padded, dried, framed, cut, creased, pressed and cured as in Example 1. The data obtained on each of the fabric samples relating to wash-and-wear, crease retention and soil release (both originally and upon restraining) appear in the accompanying Table 2. It should be noted that combining the fluorocarbon polymer and the polyether additive results in a synergistic increase in durability of the soil release as compared to that of the individual components shown in Example 1.

TABLE 2

| Percent OWF <sup>1</sup> | Monomethyl<br>ether of<br>PEG | Wash<br>and<br>wear<br>(5L-TD) | Crease<br>retention<br>(5L-TD) | Soil release    |   |   |   |                  |     |   |     |
|--------------------------|-------------------------------|--------------------------------|--------------------------------|-----------------|---|---|---|------------------|-----|---|-----|
|                          |                               |                                |                                | Original stains |   |   |   | Stained after 5L |     |   |     |
|                          |                               |                                |                                | V               | L | V | L | V                | L   | V | L   |
| 0.18                     | 5.4                           | 4.0                            | 4.0                            | 5               | 5 | 5 | 5 | 3/4              | 4   | 4 | 5   |
| 0.14                     | 5.4                           | 4.0                            | 3.5                            | 5               | 5 | 5 | 5 | 4                | 3/4 | 5 | 4/5 |
| 0.18                     | 3.6                           | 3.5                            | 4.0                            | 5               | 5 | 5 | 5 | 2/3              | 3/4 | 3 | 4   |
| 0.14                     | 3.6                           | 4.8                            | 4.5                            | 5               | 2 | 5 | 3 | 3                | 4   | 3 | 5   |

<sup>1</sup> Same concentration of dimethylol ethylene urea and zinc nitrate as in Example 1.

for 5 minutes. The dried fabric is cut into samples designated as shown in Table 1. Each sample was pressed with a crease in it on a garment press set at 100 lbs./sq. inch using the following cycle of 5 seconds steam, 10 seconds

<sup>1</sup> Polyethylene glycol (PEG) molecular weight 660, and the monomethyl ether of polyethylene glycol (MME of PEG) molecular weight 660.

70 A soil-release finish utilizing a mixture of fluorocarbon 218 polymer and polyethylene glycol MW 660

In this example the same polyester-cotton fabric substrate, durable-press resin precursor, acid catalyst and fluorocarbon polymer used in the preceding examples

## EXAMPLE 3

were used. Padding, framing, drying, cutting, creasing, pressing and curing were identical to those described in Examples 1 and 2. The concentration of the durable-press resin precursor and zinc nitrate catalyst in the bath (OWB) are identical to Examples 1 and 2. However, polyethylene glycol MW 660 was used as the polyether derivative.

As can be seen by the accompanying table, excellent and durable soil release was obtained using the synergistic mixture of the soil-release components.

in providing a durable soil-release finish, combining the same components apparently creates a synergistic mixture which imparts an effective and durable finish to the treated substrate.

As this specification discloses, numerous modifications and changes in constituents, temperatures, concentrations, substrates and the like can be made without departing from the inventive concept. The metes and bounds of this invention are best determined by the claims which follow, read in conjunction with the specification.

TABLE 3

| Percent OWF <sup>1</sup> | Fluorocarbon polymer-active | Polyethylene glycol (Carbowax 1540) | Wash and wear | Grease retention (5L-TD) | Soil release    |    |     |    |                  |     |    |    |     |
|--------------------------|-----------------------------|-------------------------------------|---------------|--------------------------|-----------------|----|-----|----|------------------|-----|----|----|-----|
|                          |                             |                                     |               |                          | Original stains |    |     |    | Stained after 5L |     |    |    |     |
|                          |                             |                                     |               |                          | 1L              | 2L | 1L  | 2L | 1L               | 2L  | 1L | 2L |     |
| 0.18-----                |                             | 5.4                                 | 4.0           |                          | 4.3             | 5  | 5   | 5  | 5                | 3/4 | 4  | 5  | 5   |
| 0.14-----                |                             | 5.4                                 | 4.0           |                          | 4.3             | 5  | 5   | 5  | 5                | 4/5 | 4  | 5  | 5   |
| 0.18-----                |                             | 3.6                                 | 4.0           |                          | 4.3             | 5  | 2/3 | 5  | 4/5              | 4   | 3  | 5  | 5   |
| 0.14-----                |                             | 3.6                                 | 4.0           |                          | 4.5             | 4  | 2/3 | 5  | 3/4              | 3   | 2  | 4  | 3/4 |

NOTE.—See footnotes bottom of Table 1.

## EXAMPLE 4

Soil-release compositions utilizing the fluorocarbon polymer durable-press resin precursor, acid catalyst of Examples 1 to 4 admixed with different polyether derivatives

Pad bath formulations are prepared containing OWB: 30  
9.5% dimethyloldihydroxyethylene urea  
1.0% fluorocarbon polymer of embodiment A  
1.0% zinc nitrate, and  
10% of the following polyether derivatives:

|                                           | MW   | 35 |
|-------------------------------------------|------|----|
| Monoooleate of polyethylene glycol -----  | 660  |    |
| Monoooleate of polyethylene glycol -----  | 860  |    |
| Monoooleate of polyethylene glycol -----  | 1260 |    |
| Monoooleate of polyethylene glycol -----  | 3610 | 40 |
| Dioleate of polyethylene glycol -----     | 1070 |    |
| Dioleate of polyethylene glycol -----     | 3870 |    |
| Monostearate of polyethylene glycol ----- | 3610 |    |
| Distearate of polyethylene glycol -----   | 3870 |    |

Padding, wet pickup, drying, framing, sampling, creasing, pressing, etc. are identical to the preceding examples.

In each instance, good, durable soil-release finishes are obtained which do not impair the durable-press finish.

As the preceding discussion and examples indicate, the results obtained by the practice of this invention are both 50 advantageous and unexpected.

For example, both durable stain release are obtained in fabrics and garments containing natural or synthetic fibers or their blends. Furthermore, unlike the soil-release compositions claimed in U.S. Pat. No. 3,377,249 to Marco, oily soil can be completely removed in a single laundering rather than requiring several launderings. In addition neither the quality or durability of the durable-press finish is compromised by the novel soil-release finishes of this invention.

The finding that effective and durable soil-release finishes could be obtained by treatment with compositions free from acrylic acid type polymers was particularly surprising in view of the disclosure of the recently issued Marco patent, which teaches that not only are acrylic acid type polymers required, but that compositions containing less than 20% by weight of acrylic acid type components were ineffective and commercially unacceptable. This fact, coupled with applicants' finding that complete soil release of oily stain could be effected in only one laundering as compared to the several required by Marco, was wholly unexpected. A further unusual aspect to applicants' invention is the discovery that while the individual components of the soil-release finish, fluorocarbon polymer, polyether derivative are individually ineffective

25 We claim:

1. A process for imparting both soil-release and durable-press characteristics to a fabric containing a blend of cellulosic and polyester fibers, said process comprising applying to each 100 parts by weight of said fabric

(1) from about 0.1 to 3.0 parts by weight of a fluorocarbon homopolymer wherein said fluorocarbon homopolymer is prepared from a monomer of the formula



wherein

$\text{R}'_1$  is a perfluoroalkyl radical having 6 to 10 carbon atoms,

$\text{R}^2$  is hydrogen or alkyl of from 1 to 6 carbon atoms,  $d$  is an integer of from 12 to 20, and

$\text{R}^3$  and  $\text{R}^4$  are selected from the group consisting of hydrogen and lower alkyl having from 1 to 4 carbon atoms.

25 2. from about 2 to 15 parts by weight of at least one 55 polyether derivative selected from the group consisting of polyalkylene glycol and esters, and ethers of said polyalkylene glycol,

3. from about 3.0 to 20 parts by weight of an acid 60 catalyzed durable-press resin precursor which is an adduct of formaldehyde and an amide, and,

4. from about 0.1 to 5.0 parts by weight of an acidic catalyst for said durable-press resin precursor, and heating the textile material until the durable-press resin precursor is cured and a soil-release and durable-press 65 finish is imparted to the fabric.

2. A process as claimed in claim 1 wherein the polyether derivative is polyethylene glycol, a fatty acid ester of polyethylene glycol or an alkyl ether of polyethylene glycol.

3. A process as claimed in claim 1 wherein said durable-press resin is cured by heating at a temperature of about 130° C. to 200° C.

4. A process as claimed in claim 1 wherein 0.15 to 0.5 part by weight of fluorocarbon homopolymer are applied to each 100 parts by weight of textile material.

5. A process as claimed in claim 3 wherein said fluorocarbon homopolymer is a homopolymer of a monomer having the formula



and said polyether derivative is selected from the group consisting of polyethylene glycol, monomethyl ether of polyethylene glycol, monooleate of polyethylene glycol, dioleate of polyethylene glycol, monostearate of polyethylene glycol and distearate of polyethylene glycol.

## References Cited

## UNITED STATES PATENTS

- |             |         |                      |             |
|-------------|---------|----------------------|-------------|
| 2,915,554   | 12/1959 | Ahlbrecht et al. --- | 260—86.1X   |
| 3,377,249   | 4/1968  | Mario -----          | 260—29.4UXL |
| 5 3,462,296 | 8/1969  | Raynolds et al. ---  | 260—29.6X   |

JULIUS FROME, Primary Examiner

J. B. LOWE, Assistant Examiner

U.S. CL. X.R.

117—139.4; 260—29.4UA, 29.6F